

## UNITED STATES PATENT OFFICE

KIRKE L. MOSES, OF BROOKLINE, MASSACHUSETTS

## PAPER-LIKE PRODUCT AND METHOD OF MAKING THE SAME

No Drawing.

Application filed March 2, 1925. Serial No. 12,590.

This invention relates to the sort of products obtained when an absorbent paper base is saturated or impregnated with various liquids such as liquids containing rubber and water (which embrace, among others, natural rubber, balata or gutta-percha containing latices preserved with ammonia, or dispersions, suspensions or emulsions of rubber involving water, all of which may be classified 5 as aqueous liquid containing rubber or aqueous dispersions of rubber); gelatine, glue and glycerine containing liquids; and drying-oil containing emulsions, and aims to facilitate the application of the before-mentioned water containing materials to the paper web.

Some of the characteristics of the products so obtained are an increased tensile strength, an increased tear resistance, an increased folding number, an increased resistance to an 20 abrasive action, etc. The degrees of increase of strength and the increase along any particular line depends on the character of the filling material which is used. For instance, if the filling material is one containing rubber 25 the resultant product will have a considerably increased folding resistance and also an increased resistance to abrasion. While papers impregnated with gelatine and glycerine have many of the characteristics common to 30 the papers impregnated with the rubber material yet they fail to have the tear resistance and tensile strength when wet which is a conspicuous feature of the rubber-impregnated papers.

In order to readily obtain a high degree 35 of impregnation it is an advantage to use a highly-porous loosely-matted paper, but heretofore this has not been practical because of the difficulty of preventing such paper 40 from tearing apart when it becomes wet during the impregnation process. Heretofore it has been found necessary to use for this purpose a paper web which is more or less absorbent but which depends for its strength 45 while wet during the impregnating operation either upon a closer matting of its own fibres than is desirable or upon its fibres being of generous length with consequent greater entanglement to enable it to pass through the 50 impregnating solution without danger of be-

ing torn apart. In the first case the closer matting of the fibres is naturally accompanied by a loss of porosity that makes impregnation operations with some of the before-mentioned materials difficult or impossible. 55 A paper as commonly made for saturating purposes in either of the foregoing ways leaves much to be desired for porosity and/or speedy handling when wet, so that much economy in its subsequent processing has 60 heretofore been sacrificed.

This invention contemplates making available for saturation and manipulation when in a wet state papers of more loosely-matted structure and shorter fibre than are considered practical at present.

This object may be obtained by mixing with the paper-making fibre in the beater, or before it is formed into a web, a material calculated to give wet strength by lightly 70 attaching the paper fibres together in the final porous web with a water insoluble or water resistant binder, and then forming by a paper-making process a loosely-matted highly-porous web which, when dry, has its fibres lightly attached by a constituent which imparts conspicuous strength when the web is re-wet during subsequent processing. It is not essential that the water resistant constituent be uniformly distributed throughout 75 the mass of the web so that all fibres are attached to their neighbors, as it is sufficient if the distribution of such constituent is more or less spotty. And by the term "lightly attached" as used in the specification and claims 80 I intend to cover either an attachment which more or less uniformly affects all the fibres of the web or is dotted irregularly throughout the mass of the web.

Among the various strength-giving elements which may thus be used to lightly attach the fibres of the porous sheet together may be mentioned viscose, rosin size, animal size, casein etc.

The viscose for this purpose may vary in 90 character depending on the source of cellulosic material from which it is manufactured. It is not necessary that it should be of a character in which there is complete conversion 95 of the cellulosic material to cellulose xan-

55

60

65

65

70

75

80

85

90

95

100

thatate or diocarbonate (i. e. viscose), as a viscose which contains a percentage of cellulosic material only partially converted will answer the purpose of this invention.

5 An advantage which is gained by the use of viscose, whether completely or partially converted, is that the viscose will act without the necessity of adding a precipitant to the material in the beater. When viscose containing fibre is used the partially converted fibres of the viscose mingle with the paper fibres and form a network of adhesive fibres throughout the paper fibres and serve to lightly bind them together with a water resistant medium, and without the addition of a precipitant. On the other hand, where rosin size or animal size or casein or some other strength-giving elements are used it is desirable to add a precipitant so as to precipitate some of the size on the paper fibres. When viscose, which, as its name implies, is of a highly viscous and sometimes jell-like nature, is added to a large quantity of water and mixed therewith, it will not be uniformly dissolved by the water, but, instead, will break up into small jell-like particles. Hence, when viscose is added to paper-making material, these jell-like particles become distributed spottily throughout the fibre mass before it is formed into paper. When, therefore, the paper is made, these jell-like particles are distributed throughout the web, and when they become dry, by the drying of the paper, they form a water-resistant binder which lightly attaches the fibres together, this result being accomplished without the use of a precipitant. Any other sizing having a jell-like nature and which, like viscose, does not dissolve in the water, but, instead, breaks up into small jell-like particles, has the same advantages as viscose and comes within the scope of the present invention.

45 My invention contemplates the use of any of these strength-giving elements in a relatively small quantity which while sufficient to cause the paper fibres to be lightly attached and thereby impart the desirable wet strength to the web, is not, however, in sufficient quantity to effect appreciably the desirable high porosity of the web.

55 A paper web made according to the above method is substantially as porous as one which is produced from the same stock without the addition of the strength-giving element but it is appreciably stronger than paper made in the same way and of the same fibre but without the addition of this strength-giving constituent. The extra strength which is inherent in paper made in accordance with this invention is particularly conspicuous while the paper, when in a wet condition, is being subjected to the manipulation necessary to impregnate it with an aqueous liquid containing rubber or an aqueous dispersion of rubber or, in other

words, with materials containing water, such for instance as rubber, gutta percha, or balata containing latex preserved with ammonia; or emulsions or dispersions or suspensions of rubber involving water; or glycerine additions to glue or gelatine or isinglass; or casein and water; or oil emulsions.

70 A wide variety of the usual rubber compounding and/or vulcanizing ingredients may be used in the above-mentioned rubber-containing liquids, also various hardening and insolubilizing agents, such as formaldehyde, parafform and the like may be used in conjunction with the glue, gelatine or casein 75 solutions.

80 My invention is to be distinguished from the ordinary process of sizing paper and from the ordinary conception of the results of sizing paper. The purpose in view in sizing paper, as it is ordinarily carried out in paper-making operations, is to introduce into the paper either a loading material to render the paper solid and less porous, or a make-weight, or for the purpose of giving the 85 paper a better finish or sometimes when used in a large quantity to give the paper water resistant qualities. Another purpose of size, particularly rosin size, is to help retention of substantial quantities of such loading and 90 filling materials as clay, etc.

95 In all of the ordinary sizing operations of paper, some of which have been above referred to, the ultimate intention or effect is to render the paper less porous by filling 100 to a greater or less extent the interstices between the fibres, and to stiffen and/or solidify the sheet. A calendering operation is generally used in conjunction with size to assist it to this end. On the other hand, the contemplation of this invention is a novel use of size with results quite opposed to the heretofore practice and generally understood function of size, for it is the purpose of my invention to add the strength-giving 105 element solely for the purpose of increasing the wet strength of paper of any fibre length and to do this without appreciably affecting the extremely novel high porosity of the paper advantageous to allow free entrance 110 of such materials as rubber containing latex.

115 While the percentage of strength-giving element which is used will vary somewhat with the character of the size I have found good results are obtained by using approximately 5% or less to the final paper web by weight of viscose. Approximately the same percentage of other kinds of sizing will suffice.

120 The present invention makes it possible to handle a wet highly-porous loosely-matted web at increased speed over present methods and under the tension which may be desirable or necessary in carrying out the impregnation of said papers in large scale 125 130

operations and without danger that the web will be broken or torn apart with a consequent process interruption.

Heretofore, as far as is known, papers intended for saturation operations have not contained anything in the nature of a size, for in paper-making practice size is supposed and/or intended to eliminate or lessen porosity and absorbency. Because these 10 characteristics are obvious requisites to a desirable saturating paper, size has not entered their make up in the past for fear of detracting from these qualities.

A web of loosely-matted fibres with high 15 porosity made in accordance with this method differs from ordinary paper in being soft to the touch, is not stiff or tinny, has no crackle, and is felt-like in structure and noticeably tender. Although the web is 20 formed by a paper-making process it is not a paper of commerce for none of the ordinarily practised uses of paper can be economically made of it, and it should not even be confused with blotting paper, which latter is 25 absorbent and more or less porous but does not contain water resistant or insoluble size and, therefore, does not have sufficient wet strength for the purposes described. This loosely-matted highly-porous paper-like web 30 is designed solely for use as a component or base of the product obtained after it has later been treated with various water containing solutions which after drying alter its original characteristics.

35 The manipulation of the web when in a wet state, which is referred to in the above description and the claims, is the manipulation to which it is necessary to subject the web during the saturation or impregnation process.

40 The word "latex" as used herein is intended to include the aqueous dispersions of rubber or the aqueous liquids containing rubber, some of which are mentioned above, whether 45 or not said liquids have compounding or vulcanizing ingredients mixed therewith.

I claim:

1. The process of making a paper-like product which consists in forming by a 50 paper-making process an absorbent web of loosely-matted fibres, increasing the wet strength of the web to a point where it will hold together when manipulated in a wet state by incorporating in the material of 55 which the web is constituted a water resistant wet-strength giving ingredient which acts to lightly bind the fibres together when the web is wet but which does not appreciably affect the porosity of the web; then impregnating 60 said web with rubber containing latex and evaporating water therefrom.

2. The process of making a paper-like product which consists in forming by a paper-making process a highly-porous web of loosely-matted fibres which are lightly attached 65

together with sufficient viscose to hold the fibres together when the web is wet, then impregnating said web with aqueous liquid containing rubber and evaporating water therefrom.

3. A paper product comprising a porous base of loosely-matted fibres which are lightly attached together with viscose, said base being impregnated with aqueous liquid containing rubber.

4. A paper product comprising a porous base of loosely-matted fibres, which are lightly attached together with sufficient viscose to hold the fibres together when the porous web is wet, said base being impregnated with rubber.

5. A paper product comprising a base of loosely-matted fibres which are attached together with sufficient viscose to hold the fibres of the base together when the latter is wet, said base being impregnated with the solid constituents of latex.

6. A paper product comprising a porous base of loosely-matted fibres, which base of itself has a wet strength below that required to prevent the base from tearing when it is manipulated while in a wet condition, said fibres being lightly attached together by water-resistant material which imports into the base sufficient strength to prevent the web from tearing apart when manipulated in a wet state, said base being impregnated with a filling material which toughens the base.

7. A paper product comprising a porous base of loosely-matted fibres, which base of itself has a wet strength below that required to prevent the base from tearing when it is manipulated while in a wet condition, said fibres being lightly attached together by water-resistant material which imports into the base sufficient strength to prevent the web from tearing apart when manipulated in a wet state, said base being impregnated with the solid constituents of latex.

8. A paper-like product comprising a base in the form of a web of fibres so loosely matted together that of themselves they are not capable of maintaining the integrity of the web when wet, said fibres being lightly attached together by a sufficient quantity of water-resistant material to prevent the web from tearing apart when manipulated in a wet state, the said base having these characteristics being impregnated with the solid constituents of latex.

In testimony whereof, I have signed my name to this specification.

KIRKE L. MOSES.

125

130